# EUROPEAN PATENT SPECIFICATION

(11) **EP 2 818 578 B1**
(45) Date of publication and mention of the grant of the patent: **22.08.2018**
(21) Application number: 13751445.1
(22) Date of filing: 21.02.2013
(51) Int. Cl.: C25F 3/06

(54) **METAL MATERIAL SURFACE TREATMENT METHOD, AND METAL MATERIAL**
OBERFLÄCHENBEHANDLUNGSVERFAHREN FÜR METALLMATERIAL UND METALLMATERIAL
PROCÉDÉ DE TRAITEMENT DE LA SURFACE D'UN MATÉRIAU EN MÉTAL ET MATÉRIAU EN MÉTAL

(30) Priority: 24.02.2012 JP 2012038556; 24.02.2012 JP 2012038560
(43) Date of publication of application: 31.12.2014
(73) Proprietor: JFE Steel Corporation, Tokyo, 100-0011 (JP)
(72) Inventor: NAGOSHI, Masayasu, Tokyo 100-0011 (JP); SATO, Kaoru, Tokyo 100-0011 (JP); BABA, Kazuhiko, Tokyo 100-0011 (JP); NORO, Hisato, Tokyo 100-0011 (JP); WATANABE, Seiichi, Sapporo-shi Hokkaido 060-8628 (JP); YOSHIDA, Souki, Sapporo-shi Hokkaido 060-8628 (JP)
(74) Representative: Stebbing, Timothy Charles
(86) International application number: PCT/JP2013/054412
(87) International publication number: WO 2013/125657

(56) References cited:
- EP-A1- 2 112 670
- WO-A1-02/33147
- WO-A1-2010/092579
- JP-A- H04 136 198
- JP-A- H04 136 198
- JP-A- 2004 512 430
- JP-B- S4 218 043
- US-A- 4 828 665
- US-A- 5 700 366

## Description

### Field

The present invention relates to a metal material surface treatment method to add a new function to the surface of the metal material and relates to a metal material subjected to surface treatment by the surface treatment method.

### Background

When the surfaces of metal materials are utilized as functional materials, an important factor is wettability of the surfaces of the metal materials, in other words, hydrophilicity and water repellency of the metal materials. Various characteristics can be imparted to metal materials by controlling the factor. For example, metal materials used for heat exchangers require an affinity between a medium such as water and the inner and outer surfaces of the metal heat exchanger tube, in other words, wettability of the surfaces of the metal materials, to increase heat conduction. Imparting hydrophilicity to the surfaces provides many advantages, for example, that self-cleaning effect of washing deposit of dirt and the like away with water can be expected. Techniques to impart hydrophilicity to metal surfaces are thus disclosed as follows: for example, Patent Literature 1 discloses a technique to form a porous oxide layer using corona discharge; and Patent Literature 2 discloses a method of forming a hydrophilic film by etching a surface to form a film thereon and then removing the film.

However, the technique using corona discharge is a technique to form an oxide layer on a surface, and once the oxide layer has removed due to peeling or the like, the function disappears. The method in which a hydrophilic film is combined with etching is expensive because of its complicated processes involving film formation. Moreover, once the hydrophilic coating has removed in use, the effect decreases and is not recovered, for example. On the other hand, as for water repellency on the surfaces of metal materials, for example, metal materials such as steel materials react with water to corrode in an environment containing water. Water repellency imparting techniques to prevent metal materials from corroding have been thus proposed in recent years. In the techniques, the surfaces of the metal materials are formed to have water repellency (hydrophobicity), which reduces wet areas on the surfaces of the metal materials or allows water in contact with the metal surfaces to readily run off the metal surfaces.

For example, Patent Literature 3 discloses a technique to impart water repellency to the surface of a steel sheet by applying an alkoxide of Al, Zr, or another element onto the surface of the steel sheet and heating the surface at 100°C or higher. Patent Literature 4 discloses a technique to impart water repellency to the surface of a plated steel sheet by forming a coating layer of a compound for metal coupling treatment on the surface of the plated steel sheet. Patent Literature 5 discloses a technique to impart water repellency to the surface of a metal sheet by applying a water repellent coating onto the surface of the metal sheet. However, all of the above methods relate to the formation of a film on the surface using an expensive agent. This leads to disadvantages such that when such a film layer has removed due to peeling or the like, water repellency thereof is impaired, and that the process of forming the film is complicated and expensive.

In recent years, in addition to various kinds of innate performance of steel sheets, attempts have been made to add new functions to steel sheets, such as dirt resistance and deodorization properties, using photocatalysts (see Patent Literatures 6 to 9). The basic technique of such attempts is to disperse photocatalyst active particles in a coating material at a surface or in a process layer. Resin materials (see Patent Literatures 6 and 7) and an inorganic-organic composite (see Patent Literature 8) have been proposed as such a coating material. Disclosed as an attempt to directly add photocatalysts to steel sheets is a technique to produce a TiO₂ thin film on the surface of a steel sheet by a film formation method in an atomic level using plasma (plasma-enhanced atomic layer deposition) (see Non-Patent Literature 1).

Patent Literature 10 discloses a method in accordance with the preamble of claim 1, in which the voltage is gradually increased whilst measuring the current so as to obtain a "bubble" regime where the current decreases or at least does not increase significantly with increase in voltage.

Patent Literature 11 discloses electroplating by varying a voltage applied between an electrode and a material to be plated so as to obtain a plating layer with a continuous variation of color tone and gloss.

Other relevant disclosures are contained in Patent Literatures 12 to 14.

### Citation List

### Patent Literature

Patent Literature 1: Japanese Laid-open Patent Publication No. 05-179419
Patent Literature 2: Japanese Laid-open Patent Publication No. 2002-053977
Patent Literature 3: Japanese Laid-open Patent Publication No. 01-068477
Patent Literature 4: Japanese Laid-open Patent Publication No. 09-020983
Patent Literature 5: Japanese Laid-open Patent Publication No. 2008-075064
Patent Literature 6: Japanese Laid-open Patent Publication No. 2000-014755
Patent Literature 7: Japanese Laid-open Patent Publication No. 2001-131768
Patent Literature 8: Japanese Laid-open Patent Publication No. 2007-268761
Patent Literature 9: Japanese Laid-open Patent Publication No. 2002-053978
Patent Literature 10: US 5 700 366 A
Patent Literature 11: JP H04 136198 A
Patent Literature 12: WO 2010/092579 A1
Patent Literature 13: WO 02/33147 A1
Patent Literature 14: US 4 828 665 A

### Non Patent Literature

Non Patent Literature 1: Chang-sooLee et al., Thin Solid Films, 518 (2010) pp.4757 - 4761

### Summary

### Technical Problem

The conventional hydrophilicity imparting techniques and water repellency imparting techniques are techniques to impart hydrophilicity and water repellency, respectively, to metal surfaces by forming films on the surfaces of metal materials. It is necessary for these techniques to add dissimilar metals or fine particles to the metal surfaces, which requires additional labor and cost. In addition, as for water repellency, it is insufficient to simply provide a water repellent layer onto the surface of a metal material, and special treatment is needed to be performed, such as addition of fine particles.

The conventional photocatalyst function imparting technique adds a photocatalyst function to the surfaces of steel sheets by dispersing photocatalyst active particles in a coating material or a process layer or forming a film of a photocatalyst active substance. However, the coating material and the process layer that mainly contain organic substances are decomposed with the photocatalyst active particles, and thus, the photocatalyst function cannot be expected to continue for a long time. Moreover, the use of photocatalyst active substances and organic materials leads to complicated production steps, which results in high cost. The film formation method of a TiO₂ thin film in an atomic level needs advanced technique and high cost, and thus it is difficult to industrialize the method.

In view of the above, it is an object of the present invention to provide a metal material surface treatment method that can add a new function to the surface of a stainless steel material without requiring a lot of labor and high costs, and a stainless steel material subjected to surface treatment by the surface treatment method.

### Solution to Problem

A metal material surface treatment method according to the present invention includes: immersing, in an electrolyte solution, a target material as a cathode electrode that is made of a stainless steel material and that has a target surface, and an anode electrode; applying a first voltage between the cathode electrode and the anode electrode; and applying a second voltage different from the first voltage between the cathode electrode and the anode electrode; characterized in that fine projections are formed on the target surface of the stainless steel material by applying the first voltage and the second voltage.

In the above-described metal material surface treatment method according to the present invention, the first voltage is 70 V or more and in a voltage range in which the cathode electrode is not oxidized or does not melt, and the second voltage is in the voltage range and differs from the first voltage by 5 V or more.

In the above-described metal material surface treatment method according to the present invention, the first voltage is 60 V or more and in a voltage range in which the cathode electrode does not melt, and the second voltage is in the voltage range and differs from the first voltage by 5 V or more.

In the above-described metal material surface treatment method according to the present invention, the second voltage is lower than the first voltage.

The above-described metal material surface treatment method according to the present invention further includes performing one or more times of treatment at a voltage lower than the second voltage by 5 V after treatment at the applying of the second voltage, and the voltage in the later treatment is lower by 5 V or more than the voltage in the immediately preceding treatment.

The above-described metal material surface treatment method according to the present invention further includes performing water repellent treatment on a surface of the cathode electrode after the applying of the first voltage and the applying of the second voltage.

A stainless steel material according to the present invention is subjected to surface treatment by the metal material surface treatment method according to the above-described present invention.

### Advantageous Effects of Invention

With the metal material surface treatment method and the stainless steel material according to the present invention, a new function can be added to the surface of the stainless steel material without requiring a lot of labor and high cost.

### Brief Description of Drawings

FIG. 1 is a flowchart illustrating the flow of surface treatment for a metal material according to a first embodiment of the present invention.
FIG. 2 is a schematic illustrating a configuration example of a device used in a surface treatment method of a metal material according to the first embodiment of the present invention.
FIG. 3 is a scanning electron microscope (SEM) photograph illustrating the surface of stainless steel SUS316 subjected to the surface treatment.
FIG. 4 is a photograph illustrating a state of distilled water added dropwise onto the surface of the test piece illustrated in FIG. 3, which is observed from the lateral direction.
FIG. 5 is a photograph illustrating a state of distilled water added dropwise onto the surface of the stainless steel illustrated in FIG. 3 that had been subjected to water repellent treatment, which is observed from the lateral direction.
FIG. 6 is a photograph illustrating a state of distilled water added dropwise onto the surface of stainless steel that is not subjected to the surface treatment and water repellent treatment, which is observed from the lateral direction.
FIG. 7 is a flowchart illustrating the flow of surface treatment for a metal material according to a second embodiment of the present invention.
FIG. 8 is a diagram illustrating a secondary electron image of the surface of stainless steel 316 treated at Step S12 in FIG. 7.
FIG. 9 is a diagram illustrating a secondary electron image of the surface of stainless steel 316 treated at Step S13 in FIG. 7.
FIG. 10 is a graph illustrating an example of absorbance spectra.

### Description of Embodiments

The metal material surface treatment method according to the first and the second embodiments of the present invention will be described with reference to the accompanying drawings.

### (First Embodiment)

FIG. 1 is a flowchart illustrating the flow of surface treatment for a metal material according to the first embodiment of the present invention. FIG. 2 is a schematic illustrating a configuration example of a device used in the metal material surface treatment method according to the first embodiment of the present invention. As illustrated in FIG. 1, in the surface treatment of a metal material according to the first embodiment of the present invention, first, a target material that is the metal material serving as a cathode electrode, and an anode electrode are immersed in an electrolyte solution, and a voltage A is applied between the cathode electrode and the anode electrode (Step S1). A voltage B different from the voltage A is applied between the cathode electrode and the anode electrode (Step S2). These two steps enable formation of a fine structure having a large specific surface area on the surface of the target material. More specifically, as illustrated in FIG. 2, an anode electrode 3 and a target material 4 are immersed in an electrolyte solution 2 in a container 1. The voltage A and the voltage B are applied to the anode electrode 3 and the target material 4 from a power source 6 through a conducting wire 5 such as a copper wire to form a fine structure on the surface of the target material 4. It is efficient to perform treatment at Step S1 and treatment at Step S2 in succession. However, the treatment at Step S2 may also be performed after a certain time from the treatment at Step S1 or after the device, the electrolyte solution, or the like is changed.

The electrolyte solution 2 is not particularly limited but is an electroconductive solution that is unlikely to excessively etch the surface of the target material 4, to adhere to or be deposited on the surfaces of the anode electrode 3 and the target material 4, and to form precipitates, during the surface treatment of the target material 4. Examples of an electrolyte of such an electrolyte solution 2 include potassium carbonate (K₂CO₃) sodium carbonate (Na₂CO₃), sodium hydrogencarbonate (NaHCO₃), ammonium carbonate ((NH₄)₂CO₃) lithium hydroxide (LiOH), sodium hydroxide (NaOH), potassium hydroxide (KOH), ammonium hydroxide (NH₄OH), sodium chloride (NaCl), potassium chloride (KCl), ammonium chloride (NH₄Cl; , sodium salts of sulfuric acid, potassium salts of sulfuric acid, ammonium salts of sulfuric acid, sodium salts of nitric acid, potassium salts of nitric acid, ammonium salts of nitric acid, sodium salts of citric acid such as sodium citrate (NaH₂(C₃H₅O(COO)₃)), potassium salts of citric acid, ammonium salts of citric acid, nitric acid, and hydrochloric acid.

The electrolyte solution 2 can have any pH and concentration so long as the electrolyte solution 2 can reform the surface of the target material 4. For example, when an aqueous solution of potassium carbonate is used as the electrolyte solution 2, its concentration is not particularly limited and may be 0.001 mol/L or higher and more preferably 0.005 mol/L or higher. This is because an excessively low concentration of the electrolyte solution 2 may make it difficult to maintain a favorable discharge state when voltage is applied between the anode electrode 3 and the target material 4. The upper limit of the concentration of the electrolyte solution 2 is not particularly set and may be, for example, 0.5 mol/L or lower. The pH of the electrolyte solution 2 can be any value unless the electrodes are excessively corroded or etched, and can be a pH of, for example, 10 to 12.

The anode electrode 3 is formed from a material thermally and chemically stable in electric discharge process. Examples of such an anode electrode 3 include Pt, Ir, and graphite.

The target material 4 is not particularly limited so long as it is a metal material. When the target material 4 is a steel material, a cold-rolled material, a hot-rolled material, a casting material, or a work thereof (including a welded material) can be employed. The type of the steel is not particularly limited, and plain carbon steel, low-alloy steel, stainless steel, or other steel is available. A plated steel sheet such as an electrogalvanized steel sheet is also available. The shape of the target material 4 is not particularly limited, and the target material 4 can have a form of a plate, a wire, a bar, or a pipe, or can employ a machined part. The target material 4 needs to be immersed in the electrolyte solution 2 and to be set at a place at least 1 mm lower than the liquid surface.

The available range of the discharge condition is from a partial plasma state to a full plasma state in which the surface of the target material 4 has irregularities. However, the discharge needs to be performed in a voltage range lower than a voltage at which the target material 4 melts. Specifically, the range is from a state where emission of light observable by the unaided eye starts in a dark place while the discharge voltage is increased, to a state just before where the whole material glows, via a state where a spots of orange light are emitted. When the size of the target material 4 is 1 mm × 1 mm × 20 mm, the application voltage is preferably in a range from 70 to 200 V and more desirably in a range from 80 to 150 V. This voltage range is applicable to most of steel materials including alloy steel such as stainless steel. However, the voltage range varies depending on the type and the location of the target material 4. The voltage range may be thus determined by observing the surface of the target material 4 treated at different voltage conditions, with a scanning electron microscope (SEM).

A necessary condition for the discharge voltage is to be a voltage at which fine projections are formed on the surface of a steel material. No fine projection is formed on the surface at a voltage lower than the lower limit. Thus, the presence or absence of fine projections can be determined by examining it with an SEM. When the voltage exceeds the upper limit, the target surface is melted. The voltage at which the surface melts can thus be determined as the upper limit. When oxidization of the surface is not desirable, a voltage at which the surface is oxidized can be easily determined by examination with an SEM and an energy-dispersive X-ray spectrometer (EDS) included with the SEM. The surface can be determined to have been oxidized when oxygen is detected at an X-ray intensity nearly equal to that of the oxide of the target material 4. The X-ray intensity of oxygen normalized by the Fe-L line intensity of oxygen in the target material 4 needs to be equal to or less than one third the X-ray intensity of oxygen normalized by the Fe-L line intensity of the oxide (means the oxide of Fe in case of a cold-rolled steel sheet or low alloy steel, for example) of the target material 4. The above surface examination is performed in the following manner. The target material 4 is subjected to discharge for 30 minutes at a different voltage. The target material 4 is then taken out, washed with water, and dried. The resultant target material 4 is set in an SEM for observation.

The inventors of the present invention have found that, in a desirable voltage range, fine projections enlarge in accordance with the increase in the voltage. To increase a surface area, it is advantageous to provide finer irregularities onto large irregularities, and thus, the voltage B is desirably lower than the voltage A. The voltage difference between the voltage A and the voltage B is desirably 5 V or more because the size difference of formed projections was found when the voltage A was different from the voltage B by 5 V. Furthermore, a voltage close to the upper limit of the desirable voltage range may be selected as the voltage A because it is advantageous to form large irregularities in the treatment at Step S1.

The treatment at each of Step S1 and Step S2 requires a discharge treatment time of 3 seconds or more. Although a long discharge treatment time is possible such as 60 minutes, a treatment time of 30 minutes or more is not preferable because the target material 4 may be worn if the discharge treatment time is excessively long. It is also not preferable that the discharge treatment time be long in the treatment at Step S2. This is because when the discharge treatment time increases in the treatment at Step S2, fine projections formed on the surface depend on the voltage B. The discharge treatment time may thus be 5 minutes or less in the treatment at Step S2.

FIG. 3 is an example of a treated SUS 316 stainless steel sheet having a thickness of 0.8 mm. This SUS 316 stainless steel sheet was cut into a piece having a width of 2.5 mm and a length of 30 mm and was brought into conduction via a copper wire to serve as a cathode electrode. A Pt wire having a length of 50 cm that was bended in a form of a plane without making contact with each other was used as an anode electrode. A heat-resistant resin was thermally crimped to the connecting part of the SUS 316 stainless steel sheet and the copper wire. A 20-mm long portion of the electrode was immersed in an electrolyte solution to avoid the copper wire from coming in contact with the electrolyte solution. An aqueous solution with a concentration of 0.1 mol/L of K₂CO₃ was used as the electrolyte solution. Discharge (Step S1) was performed for 10 minutes while the voltage was set to 140 V, and then, discharge (Step S2) was performed for 3 minutes while the voltage was set to 110 V. The cathode electrode was then pulled out of the electrolyte solution and was washed with water immediately thereafter.

As a result, as illustrated in FIG. 3, it was confirmed that comparatively large projections were formed on the surface of the SUS 316 stainless steel sheet, and that fine projections having an average diameter of 1 µm or smaller were formed on the comparatively large projections. It was also confirmed from elementary analysis by an EDS that the surface of the SUS 316 stainless steel sheet was not oxidized. The front end of the SUS 316 stainless steel sheet was melted away at an application voltage exceeding 160 V. This determines the upper limit of the application voltage to be 160 V. It was also confirmed from the elementary analysis by an EDS that the surface of the SUS 316 stainless steel sheet was not oxidized at an application voltage of 140 V or less. This reveals that the upper limit of the application voltage at which the surface is not oxidized is 140 V in this experiment condition and with this test material. This also determines the lower limit of the application voltage to be 80 V in view of the presence or absence of a projection structure. Accordingly, the most preferable condition as the voltage A is determined to be 140 V.

Referring back to FIG. 1, a fine structure was formed on the surface of the target material 4 in a manner as described above, and then, the target material 4 was taken out of the electrolyte solution 2 and was washed as needed (Step S3). The surface having hydrophilicity is obtained in this state. The washing is performed to remove the electrolyte solution on the surface, and examples thereof include a pure water immersion and a pure water spray processing. Pure water is not a limiting example, and a weak acid or an alkaline solution may also be used unless it damages the fine structure on the surface. During the process, electrolysis can be performed thereon. After the washing, the target material 4 may be dried, or may be treated at the following step without being dried for water repellent treatment.

FIG. 4 is a photograph illustrating a state of distilled water added dropwise onto the surface of the test piece illustrated in FIG. 3, which is observed from the lateral direction. As illustrated in FIG. 4, the contact angle is very small, which reveals that a superhydrophilic surface is obtained. The contact angle was 52 degrees when the surface was subjected to 15-minute discharge set at 140 V, the same voltage as Step S1, while the contact angle was 70 degrees when the surface was subjected to 15-minute discharge set at 110 V, the same voltage as Step S2. This reveals that two-stage treatment of treatment at Step S1 and treatment at Step S2 is required in order to attain superhydrophilicity such that the contact angle of water is around 10 degrees as illustrated in FIG. 4.

To provide a water repellent surface, the target surface of the washed target material 4 is subjected to water repellent treatment (Step S4). Examples of the available water repellent treatment method include a method of applying spray of a water repellent and a method of adsorbing an organic substance having water repellent function, such as a fluorine-based resin in a liquid phase or a vapor phase. In the present embodiment, the surface of the target material 4 was subjected to water repellent treatment by spraying Nanopro manufactured by Collonil (ingredients: a fluorocarbon resin and a silicone resin) on the surface of the target material 4 and drying it for 12 hours or longer.

FIG. 5 is a photograph illustrating a state of distilled water added dropwise onto the surface of the test piece illustrated in FIG. 3 that had been subjected to water repellent treatment, which is observed from the lateral direction. The contact angle of water was determined to be 170° through the observation, which indicates that super water repellency was achieved. The contact angle of water was 125° when a material on which no plasma discharge in solution had been performed was subjected to similar water repellent treatment. The contact angle of water was 77.2° (see FIG. 6) with a test piece to which no water repellent treatment was performed. Accordingly, it is recognized that both of the plasma discharge in solution having two stages of the treatment at Step S1 and the treatment at Step S2 and water repellent treatment are needed to provide a super water repellent surface.

The technique of the present invention to perform plasma discharge in solution in two different conditions is expandable to a technique in which plasma discharge treatment in solution is performed three or more times. Although performing treatment fewer times is advantageous in view of the time and cost required for the treatment, performing plasma discharge treatment in solution three or more times is applicable when a higher effect is required.

### (Examples)

A commercially available SUS 316 stainless steel sheet having a thickness of 0.8 mm was cut into a piece having a width of 2.5 mm and a length of 50 mm and was immersed in a diluted hydrochloric acid to be degreased. The sheet was then brought into conduction via a copper wire to serve as a cathode electrode. The upper portion of the electrode including the connecting part with the copper wire was coated with a heat-resistant resin, and the length of a target portion where the stainless steel was exposed was set to 20 mm. This electrode was immersed in an electrolyte solution. A 0.5 mmφ Pt wire having a length of 50 cm that was bended in a form of a plane without making contact with each other was used as an anode electrode. An aqueous solution with a concentration of 0.1 mol/L of K₂CO₃ was used as the electrolyte solution. The application voltage was set in a range from 110 to 140 V, and electric discharge was performed in each condition listed in Table 1. Immediately after the completion, the resultant stainless steel sheet was washed with pure water and dried. Subsequently, some of such test pieces were subjected to water repellent treatment by spraying Nanopro manufactured by Collonil onto the surfaces of the target materials, and drying the resultant target materials for 12 hours or more. Their water wettability was then examined. The water wettability was evaluated in the following manner. 1 µm of distilled water was added dropwise onto the electrode surface at six points each at regular intervals using a micropipette. The side view of the dropped water was taken using a digital camera EOS Kiss X2 manufactured by Canon Inc., and the contact angle was measured from the obtained photograph. The contact angles at the six points were averaged. The used distilled water was distilled water 049-16787 manufactured by Wako Pure Chemical Industries, Ltd. Table 1 lists the test result.

The contact angle with the surface with no treatment (Comparative Example 1) was 77°, and even when water repellent treatment was performed thereon, the contact angle increased only to 125°. In contrast, the contact angles in the examples of the present invention were 8° to 42°, indicating high hydrophilicity. The example of the present invention subjected to water repellent treatment obtained super water repellency with a maximum of 172° (Example 2). Although in comparative examples in which a single voltage is applied, the hydrophilicity was improved and the water repellency was obtained by performing water repellent treatment (Comparative Examples 2 to 13), even the most excellent contact angles were merely 52° and 147°, respectively. This reveals that treatment at two different voltages is highly effective in imparting hydrophilicity and water repellency. However, no enhancing effects were found both in hydrophilicity and water repellency in Example 6 in which the treatment time at Step S2 was 15 minutes, which was long. It is thus more preferable that the treatment time at Step S2 be 5 minutes or less.

**Table 1**

| Test number | Step S1 | | Step S2 | | Contact angle (°) | | Remarks |
|---|---|---|---|---|---|---|---|
| | Voltage (V) | Time (min) | Voltage (V) | Time (min) | No water repellent treatment | With water repellent treatment | |
| 1 | 140 | 5 | 120 | 5 | 10 | 170 | Example 1 |
| 2 | 140 | 15 | 120 | 5 | 8 | 172 | Example 2 |
| 3 | 120 | 15 | 140 | 5 | 18 | 159 | Example 3 |
| 4 | 135 | 10 | 125 | 2 | 13 | 163 | Example 4 |
| 5 | 140 | 10 | 110 | 2 | 15 | 165 | Example 5 |
| 6 | 140 | 15 | 120 | 15 | 42 | 154 | Example 6 |
| 7 | Not applied | | Not applied | | 77 | 125 | Comp. Ex. 1 |
| 8 | 110 | 2 | Not applied | | 75 | 130 | Comp. Ex. 2 |
| 9 | 110 | 15 | Not applied | | 70 | 138 | Comp. Ex. 3 |
| 10 | 125 | 2 | Not applied | | 72 | 135 | Comp. Ex. 4 |
| 11 | 125 | 15 | Not applied | | 63 | 143 | Comp. Ex. 5 |
| 12 | 140 | 5 | Not applied | | 57 | 140 | Comp. Ex. 6 |
| 13 | 140 | 15 | Not applied | | 52 | 144 | Comp. Ex. 7 |
| 14 | 140 | 20 | Not applied | | 53 | 146 | Comp. Ex. 8 |
| 15 | 140 | 30 | Not applied | | 52 | 147 | Comp. Ex. 9 |
| 16 | 120 | 5 | Not applied | | 65 | 139 | Comp. Ex. 10 |
| 17 | 120 | 15 | Not applied | | 65 | 138 | Comp. Ex. 11 |
| 18 | 120 | 20 | Not applied | | 64 | 136 | Comp. Ex. 12 |
| 19 | 120 | 30 | Not applied | | 66 | 139 | Comp Ex. 13 |

### (Second Embodiment)

The inventors of the present invention have extensively studied to add a photocatalyst function to stainless steel materials by a simple method without using TiO₂. As a result, they have found that a structure with fine irregularities is produced on the surface of a stainless steel material by subjecting the stainless steel material to plasma treatment in an electrolyte solution, thereby adding the photocatalyst function to the stainless steel material. The inventors of the present invention also have found that the photocatalyst function of a stainless steel material is significantly increased by subjecting the stainless steel material to plasma treatment twice at different voltages.

FIG. 7 is a flowchart illustrating the flow of surface treatment for a metal material according to the second embodiment of the present invention. A treatment device used in the metal material surface treatment method of the second embodiment of the present invention has the same configuration as that of the treatment device illustrated in FIG. 2. As illustrated in FIG. 7, in the surface treatment of a metal material according to the second embodiment of the present invention, first, a target material that is made of a stainless steel material and has a target surface, which serves as a cathode electrode, and an anode electrode are immersed in an electrolyte solution (Step S11). The voltage A that is 60 V or more and in a voltage range in which the cathode electrode does not melt is applied between the cathode electrode and the anode electrode to form a fine structure on the surface of the target material (Step S12). Specifically, as illustrated in FIG. 2, the anode electrode 3 and the target material 4 are immersed in the electrolyte solution 2 in the container 1. The voltage is applied to the anode electrode 3 and the target material 4 from the power source 6 through the conducting wire 5 such as a Cu wire and a Pt wire to form a fine structure on the surface of the target material 4. FIG. 8 is a diagram illustrating a secondary electron image of the surface of the stainless steel 316 treated at Step S12. As illustrated in FIG. 8, fine irregularities are formed on the surface of the stainless steel 316 treated at Step S12.

The electrolyte solution 2 is not particularly limited but is an electroconductive solution that is unlikely to excessively etch the surface of the target material 4, to adhere to or be deposited on the surfaces of the anode electrode 3 and the target material 4, and to form precipitates, during the surface treatment of the target material 4. Examples of an electrolyte of such an electrolyte solution 2 include potassium carbonate (K₂CO₃) sodium carbonate (Na₂CO₃), sodium hydrogencarbonate (NaHCO₃), ammonium carbonate ((NH₄)₂CO₃), lithium hydroxide (LiOH), sodium hydroxide (NaOH), potassium hydroxide (KOH), ammonium hydroxide (NH₄OH), sodium chloride (NaCl), potassium chloride (KCl), ammonium chloride (NH₄Cl), sodium salts of sulfuric acid, potassium salts of sulfuric acid, ammonium salts of sulfuric acid, sodium salts of nitric acid, potassium salts of nitric acid, ammonium salts of nitric acid, sodium salts of citric acid such as sodium citrate (NaH₂ (C₃H₅O (COO)₃)), potassium salts of citric acid, ammonium salts of citric acid, nitric acid, and hydrochloric acid.

The electrolyte solution 2 can have any pH and concentration so long as the electrolyte solution 2 can reform the surface of the target material 4. For example, when an aqueous solution of potassium carbonate is used as the electrolyte solution 2, its concentration is not particularly limited and may be 0.001 mol/L or higher and more preferably 0.005 mol/L or higher. This is because an excessively low concentration of the electrolyte solution 2 makes it difficult to maintain a favorable discharge state when voltage is applied between the anode electrode 3 and the target material 4. The upper limit of the concentration of the electrolyte solution 2 is not particularly set and may be, for example, 0.5 mol/L or lower. The pH of the electrolyte solution 2 can be any value unless it excessively corrodes or etches the electrodes, and can be a pH of, for example, 10 to 12.

The anode electrode 3 is formed from a material that is thermally and chemically stable for electric discharge. Examples of such an anode electrode 3 include Pt, Ir, and graphite.

The target material 4 is a stainless steel material containing 12% by weight or more of Cr and may be any of ferritic, austenitic, and dual-phase stainless steels. Any surface finishes can be used. The shape of the target material 4 is not particularly limited, and the target material 4 can have a form of foil, a plate, a wire, a bar, or a pipe, or can employ a machined part or an assembled part. The target material 4 needs to be immersed in the electrolyte solution 2 and to be set at a place at least 1 mm lower than the liquid surface.

In the discharge condition, the available voltage range is from equal to or more than a voltage at which a partial plasma state is exhibited in which irregularities are formed on the surface of the target material 4, to a voltage at which the target material 4 does not melt. The partial plasma state indicates a state in a range from a voltage at which emission of light observable by the unaided eye starts in a dark place while the discharge voltage is increased, to a voltage before reaching a full plasma state at which spots of orange light are emitted. Specifically, the voltage range can be determined by performing electric discharge and confirming the formation of a fine structure on the surface using a SEM or other devices. The general application voltage is preferably in a range from 90 to 150 V, and is adjusted to be in this voltage range for the treatment. The applicable application time is 5 seconds to 30 minutes. The fine structure means a rough structure having projection and holes, which do not exist before the treatment.

A necessary condition for the discharge voltage is to be a voltage at which the fine structure can be formed on the surface of the target material 4. No fine structure is formed on the surface of the target material 4 at discharge voltages lower than the lower limit. The presence or absence of the fine structure can be determined by examining it with an SEM. The upper limit of the discharge voltage is determined proportional to the treatment time. In other words, in high discharge voltages, although the irregularities on the surface increase, a favorable fine structure is unlikely to be formed because melting occurs. Thus, the upper limit of the discharge voltage may be determined by predetermining a time t for the treatment and performing electric discharge for the time t while the voltage is changed, thereby confirming the formation of the fine structure using a SEM. This revealed that the photocatalyst function increases in accordance with the increase in the discharge voltage in the preferable voltage range. Accordingly, the most preferable discharge voltage is obtained by selecting a discharge voltage in the preferable voltage range close to the upper limit.

The voltage B different from the voltage A is applied between the anode electrode 3 and the target material 4 (Step S13). The treatment at these two Steps S12 and S13 (Step S1 and Step S2) enables formation of a fine structure having a large specific surface area on the surface of the target material 4. The condition of the electrolyte solution and other conditions may be changed from those at Step S12. The inventors of the present invention have found that in a desirable voltage range, a fine structure enlarges in accordance with the increase in the discharge voltage. To increase a surface area, it is advantageous to provide finer irregularities onto large irregularities. Thus, the voltage B is desirably lower than the voltage A. The voltage difference between the voltage A and the voltage B is desirably 5 V or more because size difference of formed projections has been found when the voltage A differs from the voltage B by 5 V. Furthermore, a voltage close to the upper limit of the desirable voltage range may be selected as the voltage A because it is advantageous to form large irregularities in the treatment at Step S12.

The treatment at each of Step S12 and Step S13 requires a discharge treatment time of 3 seconds or more. Although a long discharge treatment time is possible such as 60 minutes, a treatment time of 30 minutes or more is not preferable because the target material 4 may be worn if the discharge treatment time is excessively long. It is also not preferable that the discharge treatment time be long in the treatment at Step S13. This is because when the discharge treatment time increases in the treatment at Step S13, a fine structure formed on the surface depends only on the voltage B, which loses the effect of treatment at two stages. The discharge treatment time may thus be 5 minutes or less in the treatment at Step S13.

FIG. 9 is a diagram illustrating a secondary electron image of the surface of the stainless steel 316 treated at Step S13. In the example illustrated in FIG. 9, Pt was used for the anode electrode 3. Electric discharge was performed for 10 minutes in an aqueous solution of 0.1 mol/L of K₂CO₃ while the voltage A was set to 140 V, and then, electric discharge was performed for 3 minutes while the voltage B was set to 110 V. The stainless steel 316 as the target material 4 was then pulled out of the aqueous solution of K₂CO₃ and was washed with water immediately thereafter. As illustrated in FIG. 9, it is confirmed that a comparatively large projection structure is formed on the surface of the stainless steel 316, and fine projections having an average diameter of 1 µm or smaller are formed on the comparatively large projections.

A decolorization test of methylene blue was performed on the stainless steel 316 illustrated in FIGS. 8 and 9 to confirm their photocatalysis performance. This also confirmed that the stainless steel 316 illustrated in FIG. 9 had higher photocatalysis performance. This reveals that higher photocatalysis performance is obtained by performing plasma treatment twice in the electrolyte solution. This technique is expandable to a technique in which plasma discharge treatment in an electrolyte solution is performed in three or more stages. Although performing plasma treatment fewer times is advantageous in view of the time and cost required for the treatment, performing plasma discharge treatment in an electrolyte solution in three or more stages can be selected when higher photocatalysis performance is required.

### (Examples)

A commercially available SUS 316 stainless steel sheet having a thickness of 0.8 mm was cut into a piece having a width of 2.5 mm and a length of 30 mm and was immersed in a diluted hydrochloric acid to be degreased. The sheet was then brought into conduction via a copper wire to serve as a cathode electrode. The upper portion of the electrode including the connecting part with the copper wire was coated with a heat-resistant resin so that the copper wire would not come in contact with an electrolyte solution, and the length of a target portion where the stainless steel was exposed was set to 20 mm. This electrode was immersed in the electrolyte solution. A 0.5 mmφ Pt wire having a length of 50 cm that was bended in a form of a plane without making contact with each other was used as an anode electrode. An aqueous solution with a concentration of 0.1 mol/L of K₂CO₃ was used as the electrolyte solution. The application voltage was set in a range from 90 to 140 V, and electric discharge was performed in each condition listed in Table 2. Immediately after the completion, the resultant stainless steel sheet was washed with pure water and dried. As a comparative example, an untreated stainless steel sheet used as a base material was used (on which degreasing was performed by being immersed in a diluted hydrochloric acid). A decolorization test of methylene blue was performed on each of such test pieces to examine their photocatalysis performance.

The following describes the decolorization test of methylene blue. Before the decolorization test of methylene blue, an aqueous solution with a concentration of 0.1% by mass of methylene blue was singly charged into a cell. The absorbance of the aqueous solution of methylene blue was measured by an absorptiometer, type: V630 manufactured by JASCO Corporation, in which the measurement starts at a wavelength of 720 nm and ends at a wavelength of 500 nm. An absorbance peak at about 660 nm that was relatively large absorbance was determined as an absorbance A_{XS} at a wavelength (X) corresponding to the maximum absorbance, and was employed as a reference.

In the decolorization test of methylene blue, 4 ml of an aqueous solution with a concentration of 0.1% by mass of methylene blue was charged into a cell, and a test piece (such as a stainless steel sheet subjected to discharge treatment) having a size of 2.5 mm × 20 mm × 0.8 mm (sheet thickness) was immersed therein. The cell containing the aqueous solution was irradiated with ultraviolet rays (having a wavelength of 365 nm). Aluminum foil was set around the cell so that the whole cell could be irradiated with the ultraviolet rays. After the ultraviolet rays were radiated for 24 hours, the test piece was taken out of the cell. The absorbance of the remaining aqueous solution was measured in the aforementioned manner, whereby the absorbance A_{XP} at the wavelength (X) was obtained. A_{XP}/A_{XS} was determined as a change in the absorbance of the aqueous solution of methylene blue to evaluate the degree of decolorization of methylene blue. Decolorization proceeds in accordance with the decrease in the value of A_{XP}/A_{XS}, and the test piece has higher photocatalysis performance, accordingly. FIG. 10 illustrates and Table 2 lists an example of the obtained absorbance spectra and the evaluation result.

Examples 1 to 3 indicate high decolorization rates as compared with untreated stainless steel sheets (Comparative Examples 1 to 5). It is also confirmed that the performance is greatly improved with discharge performed twice at different voltages.

**Table 2**

| Test number | Step S1 | | Step S2 | | Absorbance* | Remarks |
|---|---|---|---|---|---|---|
| | Voltage (V) | Time (min) | Voltage (V) | Time (min) | | |
| 21 | - | - | - | - | 0.92 | Comp. Ex. 1 |
| 22 | 90 | 15 | - | - | 0.85 | Comp. Ex. 2 |
| 23 | 120 | 15 | - | - | 0.80 | Comp. Ex. 3 |
| 24 | 140 | 15 | - | - | 0.80 | Comp. Ex. 4 |
| 25 | 140 | 30 | - | - | 0.74 | Comp. Ex. 5 |
| 26 | 140 | 15 | 110 | 5 | 0.27 | Example 1 |
| 27 | 140 | 15 | 120 | 5 | 0.32 | Example 2 |
| 28 | 140 | 15 | 135 | 5 | 0.41 | Example 3 |

| | | | | | | |
|---|---|---|---|---|---|---|
| ^{*)} The absorbance of the aqueous solution of methylene blue after the test when the absorbance of the aqueous solution before the test was set to 1 | | | | | | |

### Industrial Applicability

The present invention provides a metal material surface treatment method that can add new function to the surface of the metal material without requiring a lot of labor and high cost, and a metal material subjected to surface treatment by the surface treatment method.

### Reference Signs List

- 1: container
- 2: electrolyte solution
- 3: anode electrode
- 4: target material (cathode electrode)
- 5: conducting wire
- 6: power source
- 7: thermometer

## Claims

1. A metal material surface treatment method, comprising:
immersing, in an electrolyte solution, a target material as a cathode electrode that is made of a stainless steel material and that has a target surface, and an anode electrode;
applying a first voltage between the cathode electrode and the anode electrode; and
applying a second voltage different from the first voltage between the cathode electrode and the anode electrode;
**characterized in that** fine projections are formed on the target surface of the stainless steel material by applying the first voltage and the second voltage.

2. The metal material surface treatment method according to claim 1, wherein
the first voltage is 70 V or more and in a voltage range in which the cathode electrode is not oxidized or does not melt, and
the second voltage is in the voltage range and differs from the first voltage by 5 V or more.

3. The metal material surface treatment method according to claim 1, wherein
the first voltage is 60 V or more and in a voltage range in which the cathode electrode does not melt, and the second voltage is in the voltage range and differs from the first voltage by 5 V or more.

4. The metal material surface treatment method according to claim 2 or 3, wherein the second voltage is lower than the first voltage.

5. The metal material surface treatment method according to claim 2 or 4, further comprising
performing one or more times of treatment at a voltage lower than the second voltage by 5 V after treatment at the applying of the second voltage, and
wherein the voltage in the later treatment is lower by 5 V or more than the voltage in the immediately preceding treatment.

6. The metal material surface treatment method according to claim 2, 4, or 5, further comprising:
performing water repellent treatment on a surface of the cathode electrode after the applying of the first voltage and the applying of the second voltage.

7. A stainless steel material obtained by being subjected to surface treatment by the metal material surface treatment method according to any one of claims 1 to 6.

## Patentansprüche

1. Oberflächenbehandlungsverfahren für Metallmaterial, umfassend:
Eintauchen in eine Elektrolytlösung eines Zielmaterials als eine Kathodenelektrode, die aus einem rostfreien Stahlmaterial hergestellt ist und die eine Zieloberfläche aufweist, und einer Anodenelektrode;
Anlegen einer ersten Spannung zwischen der Kathodenelektrode und der Anodenelektrode; und
Anlegen einer zweiten Spannung, die sich von der ersten Spannung unterscheidet, zwischen der Kathodenelektrode und der Anodenelektrode;
**dadurch gekennzeichnet, dass** feine Vorsprünge auf der Targetoberfläche des rostfreien Stahlmaterials durch Anlegen der ersten Spannung und der zweiten Spannung ausgebildet werden.

2. Oberflächenbehandlungsverfahren für Metallmaterial nach Anspruch 1, wobei
die erste Spannung 70 V oder mehr beträgt und in einem Spannungsbereich liegt, in dem die Kathodenelektrode nicht oxidiert wird oder nicht schmilzt, und
die zweite Spannung im Spannungsbereich liegt und von der ersten Spannung um 5 V oder mehr abweicht.

3. Oberflächenbehandlungsverfahren für Metallmaterial nach Anspruch 1, wobei
die erste Spannung 60 V oder mehr beträgt und in einem Spannungsbereich liegt, in dem die Kathodenelektrode nicht schmilzt, und die zweite Spannung im Spannungsbereich liegt und sich von der ersten Spannung um 5 V oder mehr unterscheidet.

4. Oberflächenbehandlungsverfahren für Metallmaterial nach Anspruch 2 oder 3, wobei die zweite Spannung niedriger ist als die erste Spannung.

5. Oberflächenbehandlungsverfahren für Metallmaterial nach Anspruch 2 oder 4, ferner umfassend Durchführen einer oder mehrerer Behandlungen bei einer Spannung, die um 5 V niedriger als die zweite Spannung ist, nach der Behandlung durch Anlegen der zweiten Spannung, und
wobei die Spannung bei der späteren Behandlung um 5 V oder mehr niedriger ist als die Spannung in der unmittelbar vorhergehenden Behandlung.

6. Oberflächenbehandlungsverfahren für Metallmaterial nach Anspruch 2, 4 oder 5, ferner umfassend:
Durchführen einer wasserabweisenden Behandlung auf einer Oberfläche der Kathodenelektrode nach dem Anlegen der ersten Spannung und nach dem Anlegen der zweiten Spannung.

7. Material aus rostfreiem Stahl, das erhalten wird, indem es einer Oberflächenbehandlung durch das Oberflächenbehandlungsverfahren für Metallmaterial nach einem der Ansprüche 1 bis 6 unterzogen wurde.

## Revendications

1. Procédé de traitement de surface de matériau de métal, comprenant :
l'immersion, dans une solution électrolytique, d'un matériau cible comme une électrode cathodique qui est composé d'un matériau d'acier inoxydable et qui comprend une surface cible, et d'une électrode anodique ;
l'application d'une première tension entre l'électrode cathodique et l'électrode anodique ; et
l'application d'une seconde tension différente de la première tension entre l'électrode cathodique et l'électrode anodique ;
**caractérisé en ce que** de fines projections sont formées sur la surface cible du matériau d'acier inoxydable par l'application de la première tension et de la seconde tension.

2. Procédé de traitement de surface de matériau de métal selon la revendication 1, dans lequel
la première tension est de 70 V ou plus et comprise dans une plage de tensions dans laquelle l'électrode cathodique n'est pas oxydée ou ne fond pas, et
la seconde tension est comprise dans la plage de tensions et diffère de la première tension de 5 V ou plus.

3. Procédé de traitement de surface de matériau de métal selon la revendication 1, dans lequel
la première tension est de 60 V ou plus et comprise dans une plage de tensions dans laquelle l'électrode cathodique ne fond pas, et la seconde tension est comprise dans la plage de tensions et diffère de la première tension de 5 V ou plus.

4. Procédé de traitement de surface de matériau de métal selon la revendication 2 ou 3, dans lequel la seconde tension est inférieure à la première tension.

5. Procédé de traitement de surface de matériau de métal selon la revendication 2 ou 4, comprenant en outre
la réalisation d'un ou de plusieurs traitements à une tension inférieure de 5 V à la seconde tension après le traitement à l'application de la seconde tension, et
dans lequel la tension dans le traitement ultérieur est inférieure de 5 V ou plus à la tension dans le traitement immédiatement précédent.

6. Procédé de traitement de surface de matériau de métal selon la revendication 2, 4 ou 5, comprenant en outre :
la réalisation d'un traitement hydrofuge sur une surface de l'électrode cathodique après l'application de la première tension et l'application de la seconde tension.

7. Matériau d'acier inoxydable obtenu en étant soumis à un traitement de surface par le procédé de traitement de surface de matériau de métal selon l'une quelconque des revendications 1 à 6.
